

# United States Patent Office

3,060,047

Patented Oct. 23, 1962

1

3,060,047

## COATING MATERIAL OF BLENDED PITCH AND TAR EMULSIONS

Olin D. Graff and Malcolm Mitchell, Indianapolis, Ind., assignors to Reilly Tar and Chemical Corporation, Indianapolis, Ind., a corporation of Indiana  
No Drawing. Filed Apr. 6, 1960, Ser. No. 20,253  
4 Claims. (Cl. 106—277)

This invention relates to a discovery that, by blending together separately prepared tar-in-water and pitch-in-water-emulsions, a coating of these blended emulsions may be applied directly to metals, such as steel, even in the absence of a primer, to obtain an outstanding protective coating. The steel does not rust under the coating.

The coating involving this invention may be applied to the metal in any suitable manner as by spraying, dipping, brushing or wiping on. The coating lends itself to normal drying at atmospheric temperatures and also to baking on the metal. A peculiarity is noted in that oily coated metal may be sprayed by or dipped in the blended emulsions and good wetting and coverage by the coating on the metal is obtained. By the term "oily coated" is meant that oil coating normally adhering on metals such as they come from rolling mills, but not any normally flowing oil.

As an example, one of the two emulsions entering into the blend constituting this invention, a roofing pitch emulsion, is prepared as follows:

A coal tar roofing pitch having the properties of a softening point cube in water (ASTM D61-38) of 140 to 155° F. and insoluble in carbon disulphide (ASTM D4-52) 15 to 30 percent, is melted down in a mix tank and is cut back with 10 percent by weight of anthracene oil. To this cut back pitch in the amount of 33 to 40 percent by weight of the final emulsion, is added a filler such as talc or ball clay, within the range of from 8 to 20 percent of the final emulsion and the temperature is maintained between 105 and 115° C.

Anthracene oil may be defined (American Wood Preservers Association P-7-58) as a coke oven tar distillate with not more than 10 percent distilling at 235° C. and not less than 65 percent distilling at 355° C.

Water is metered into an emulsion tank in quantity of from 42 to 47.2 percent by weight of the emulsion and is heated to between 80 and 90 degrees C. Powdered or pelletized powdered bentonite of from 3.2 to 4.5 percent by weight is added to the heated water and the mixture is agitated until it is a smooth paste, free of lumps, at which time the paste temperature may be in the range of from 50 to 70 degrees C.

A surface acting agent, a surfactant, is selected from one of the following:

Sodium isopropylnaphthalene sulfonate (trade name Aerosol OS)  
Polyoxyethylene sorbitan mono-oleate (trade name Tween 81)  
Sorbitan mono-oleate (trade name Span 80)  
Sorbitan monolaurate (trade name Span 20)  
Sodium salt of lignin from alkaline processes of pulping southern pine wood (trade name Indulin C)

One of these surfactants such for example, as polyoxyethylene sorbitan mono-oleate is added to either the roofing pitch-filler phase or the water-bentonite phase prior to intermixing in the emulsion tank, in the proportions of from 0.1 to 0.4 percent by weight of the final emulsion.

The filled, cut back roofing pitch as above described is slowly pumped into the mixture in the emulsion tank while great agitation is maintained. The pitch is con-

2

tinued to be pumped fully into the water-bentonite phase and the agitation is continued for at least an hour or longer to complete emulsification.

A second emulsion is prepared as follows:

5 Water in amount within the range of 38 to 44 percent by weight of the completed emulsion is brought up to a temperature of 90 degrees C.

Powdered or pelletized powdered bentonite in amount by weight in the range of 3.5 to 4.0 percent is stirred 10 or agitated into the water until a smooth paste develops.

A refined coal tar is selected having a float test consistency (ASTM D139-49) of 75-220 seconds at 50 degrees C., further identified as RT-10, RT-11, or RT-12, as outlined in specification M52-42, page 32 of part I,

15 Standard Specifications of Highway Materials, Seventh Edition 1955, by American Association of State Highway Officials. An amount of approximately 32-38 percent of the selected tar is placed in an agitator tank at a temperature ranging from 90 to 100 degrees C., to which tar

20 is first added one of the surfactants above indicated as being usable, such as the polyoxyethylene sorbitan mono-oleate, in the weight proportion of 0.1 to 0.3 percent, and secondly, a filler selected from powdered bentonite, ball clay, talc, slate flour, mica, or silica, in weight proportion of 8 to 14 percent.

25 Into the phase of water-bentonite paste ranging in temperature of from 80 to 90 degrees C., is pumped slowly the tar-filler-surfactant phase under high agitation of the intermixture until all tar is added and completely emulsified.

30 The sodium salt of lignin in the amount of 0.1 to 0.3 percent by weight of the final emulsion is added by dissolving it in dilution water. The dilution water is added in an amount varying from 5 percent to 10 percent of the final emulsion weight depending upon the consistency desired. The mixture is agitated until homogeneous.

35 Both emulsions, one at a time, can be made by separate feeding of the tar-filler and water-bentonite phases to a colloid mill.

40 These two emulsions are then ready to be intermixed or blended together to form the coating product.

45 The two emulsions are blended in the ratio of 3 parts of the first emulsion to one part of the second emulsion. The blended product is varied slightly depending upon how it is to be applied. For example, to the blended emulsion is added 0.75 percent of polyoxyethylene sorbitan mono-oleate when the product is to be applied as a spray. When the product is to be employed as a dip (metal dipped into it), 1.25 percent of either sorbitan mono-oleate or sorbitan monolaurate and 0.2 percent of sodium isopropylnaphthalene sulfonate are added to the blend.

50 The two emulsions may be added together in other proportions such as 4 to 1; 2 to 1; and 1 to 1. The 1 to 1 ratio dipped coating under impact, when baked, is less satisfactory than the 4-1, 3-1, and 2-1 ratios, while the 1-1 ratio sprayed on coating wetted the oily metal better than the 3-1 and 4-1 ratio sprayed blends. The 2-1 ratio ranks below the other ratios. The 3-1 ratio is the conventional blend.

55 Additional usable emulsions of tar are set out in the following table wherein the figures are percentages by weight of the finished emulsion.

|                                    |       |     |     |     |
|------------------------------------|-------|-----|-----|-----|
| Water                              | 38    | 40  | 40  | 44  |
| KWK Bentonite                      | 3.75  | 3.5 | 4   | 4   |
| RT 10, or RT 12 (Refined Coal Tar) | 33.75 | 37  | 38  | 32  |
| Tween 81                           | .3    | .1  | .3  | .2  |
| Filler                             | 14    | 9.3 | 8   | 14  |
| Indulin C                          | 2     | .1  | .1  | .2  |
| Dilution Water                     | 10    | 10  | 9.6 | 5.6 |

70 Additional usable emulsions of pitch are set out in

the following table wherein the figures are percentages by weight of the finished pitch emulsions:

|                        | 42   | 46   | 47.2 |
|------------------------|------|------|------|
| Water                  | 42   | 46   | 47.2 |
| Pwd. Bentonite         | 3.2  | 4    | 4.5  |
| Cut back roofing Pitch | 40   | 33   | 40   |
| Tween 81               | 1    | 2    | 3    |
| Filler                 | 14.7 | 16.8 | 8    |

Therefore it is to be seen that the discovery that two separately prepared emulsions as constituted within the ranges set forth by the foregoing examples, may be blended in the indicated proportions to give new and unexpected results as a metal coating. Coatings constituting either one alone of the tar or pitch emulsions have been employed with inferior results, but the surprise of obtaining a vastly superior coating came upon blending largely by accident the two types of the emulsions.

We claim:

1. A coating composition product comprising a blend of roofing pitch emulsion and of coal tar emulsion, wherein the roofing pitch emulsion comprises soft pitch 33 percent to 40 percent by weight of the finished pitch emulsion; water, 42 percent to 47.2 percent, bentonite 3.2 percent to 4.5 percent, filler 8 to 20 percent, surfactant 0.1 percent to 0.4 percent; and the coal tar emulsion comprises water 38 percent to 44 percent by final tar emulsion weight, bentonite 3.5 percent to 4.0 percent, filler 8 to 14 percent, tar 32 percent to 38 percent, and surfactants 0.1 percent to 0.3 percent each.
2. The product of claim 1 in which said pitch is cut back with 10 percent anthracene oil.
3. The method of making a metal coating composition which comprises heating to melting point a soft coal tar roofing pitch; cutting it back with 10 percent by

weight of anthracene oil; adding a filler in the range of 8 to 20 percent to the cut-back pitch while maintaining a temperature range of from 105-115 degrees C. as one phase; mixing into 42 percent to 47.2 percent of water by total emulsion weight in a temperature range of approximately from 80 to 90 degrees C., bentonite 3.2 to 4.5 percent of total emulsion weight and agitating until a smooth paste is formed as another phase; flowing the pitch-filler phase into said water-bentonite phase and agitating to complete an emulsion; a surfactant being added to either one of said phases before flowing together; mixing together refined coal tar at a temperature range of 90 to 100° C., from 32 to 38 percent by tar emulsion weight and a filler of from 8 to 14 percent by tar emulsion weight and a surfactant forming a tar-filler phase; mixing into water ranging in amount from 38 to 44 percent by tar emulsion weight comminuted bentonite 3.5 to 4 percent by weight as a water-bentonite phase; flowing the tar-filler phase into the water-bentonite phase ranging in temperature from 80 to 90 degrees C., and agitating until a tar emulsion is formed; and blending together the pitch and tar emulsions in ratios of from 1 to 1 to 4 to 1.

4. The method of claim 3 in which the sodium salt of lignin ranging from 0.1 percent to 0.3 percent by weight in dilution water in 5 percent to 10 percent by weight, both weights being that of the final weight of tar emulsion, is added to the tar emulsion.

References Cited in the file of this patent

UNITED STATES PATENTS

- |           |                      |               |
|-----------|----------------------|---------------|
| 2,327,882 | Gabriel et al. ----- | Aug. 24, 1943 |
| 2,712,506 | Farris -----         | July 5, 1955  |